



US009064676B2

(12) **United States Patent**  
**Sullivan et al.**

(10) **Patent No.:** **US 9,064,676 B2**  
(45) **Date of Patent:** **Jun. 23, 2015**

(54) **MICROCHANNEL PLATE DEVICES WITH TUNABLE CONDUCTIVE FILMS**

(71) Applicants: **Neal T. Sullivan**, Lunenburg, MA (US); **Steve Bachman**, North Attleboro, MA (US); **Philippe de Rouffignac**, Cambridge, MA (US); **Anton Tremsin**, Lafayette, CA (US); **David Beaulieu**, Groton, MA (US); **Dmitry Gorelikov**, Ashland, MA (US)

(72) Inventors: **Neal T. Sullivan**, Lunenburg, MA (US); **Steve Bachman**, North Attleboro, MA (US); **Philippe de Rouffignac**, Cambridge, MA (US); **Anton Tremsin**, Lafayette, CA (US); **David Beaulieu**, Groton, MA (US); **Dmitry Gorelikov**, Ashland, MA (US)

(73) Assignee: **Arradiance, Inc.**, Sudbury, MA (US)

(\*) Notice: Subject to any disclaimer, the term of this patent is extended or adjusted under 35 U.S.C. 154(b) by 0 days.

(21) Appl. No.: **13/829,108**

(22) Filed: **Mar. 14, 2013**

(65) **Prior Publication Data**

US 2013/0193831 A1 Aug. 1, 2013

**Related U.S. Application Data**

(63) Continuation of application No. 13/460,726, filed on Apr. 30, 2012, which is a continuation of application No. 12/143,732, filed on Jun. 20, 2008, now Pat. No. 8,227,965.

(51) **Int. Cl.**

**H01J 43/04** (2006.01)

**H01J 43/24** (2006.01)

(52) **U.S. Cl.**

CPC ..... **H01J 43/04** (2013.01); **H01J 43/246** (2013.01)

(58) **Field of Classification Search**

CPC ..... H01J 43/04; H01J 43/246  
USPC ..... 250/390; 313/250, 399, 400, 401,  
313/103 R, 103 CM, 104, 105 R, 105 CM,  
313/532-536

See application file for complete search history.

(56) **References Cited**

**U.S. PATENT DOCUMENTS**

3,979,621 A 9/1976 Yates  
4,780,395 A 10/1988 Saito et al.  
(Continued)

**FOREIGN PATENT DOCUMENTS**

EP 1 339 087 A1 8/2003  
IL 114278 6/1995  
(Continued)

**OTHER PUBLICATIONS**

'Final Report "Fabrication and Properties of Nanolaminates Using Self-Limiting Surface Chemistry Techniques," AFOSR Grant No. F49620-99-1-0081, Prof. Steven M. George, University of Colorado, Reported on Jul. 1, 2003 and published on Jul. 9, 2003, and a partial translation hereinafter George.\*

(Continued)

*Primary Examiner* — Thomas A Hollweg

*Assistant Examiner* — Jacob R Stern

(74) *Attorney, Agent, or Firm* — Kurt Rauschenbach; Rauschenbach Patent Law Group, LLC

(57) **ABSTRACT**

A microchannel plate includes a substrate defining a plurality of channels extending from a top surface of the substrate to a bottom surface of the substrate. A resistive layer is formed over an outer surface of the plurality of channels that provides ohmic conduction with a predetermined resistivity that is substantially constant. An emissive layer is formed over the resistive layer. A top electrode is positioned on the top surface of the substrate. A bottom electrode positioned on the bottom surface of the substrate.

**30 Claims, 10 Drawing Sheets**

280



(56)

## References Cited

## U.S. PATENT DOCUMENTS

|                   |         |                                |
|-------------------|---------|--------------------------------|
| 5,378,960 A       | 1/1995  | Tasker et al.                  |
| 5,726,076 A       | 3/1998  | Tasker et al.                  |
| 5,776,538 A       | 7/1998  | Pierle et al.                  |
| 6,045,677 A *     | 4/2000  | Beetz et al. .... 205/50       |
| 6,396,049 B1      | 5/2002  | Estrera et al.                 |
| 6,492,657 B1 *    | 12/2002 | Burlefinger et al. .... 257/10 |
| 6,522,061 B1      | 2/2003  | Lockwood                       |
| 7,025,652 B2      | 4/2006  | Heo et al.                     |
| 7,333,701 B1      | 2/2008  | Feller et al.                  |
| 7,408,142 B2      | 8/2008  | Beaulieu et al.                |
| 7,425,713 B2      | 9/2008  | Beaulieu                       |
| 7,759,138 B2      | 7/2010  | Beaulieu et al.                |
| 7,855,493 B2      | 12/2010 | Sullivan et al.                |
| 7,977,617 B2      | 7/2011  | Sullivan et al.                |
| 8,052,884 B2      | 11/2011 | Sullivan et al.                |
| 8,134,108 B2      | 3/2012  | Sullivan et al.                |
| 8,227,965 B2      | 7/2012  | Sullivan et al.                |
| 8,237,129 B2      | 8/2012  | Sullivan et al.                |
| 2003/0205956 A1   | 11/2003 | Downing et al.                 |
| 2004/0245592 A1 * | 12/2004 | Harmon et al. .... 257/438     |
| 2005/0020254 A1   | 9/2005  | Heo et al.                     |
| 2007/0012930 A1 * | 1/2007  | Liu et al. .... 257/80         |
| 2007/0131849 A1   | 6/2007  | Beaulieu et al.                |

## FOREIGN PATENT DOCUMENTS

|    |             |         |
|----|-------------|---------|
| IL | 116233      | 12/1995 |
| JP | 62-41378    | 9/1987  |
| JP | S62-254338  | 11/1987 |
| JP | 01-186731   | 7/1989  |
| JP | 03-116626   | 5/1991  |
| JP | 3-116626    | 5/1991  |
| JP | 06-060800   | 4/1994  |
| JP | 11-508359   | 7/1999  |
| JP | 3113902     | 9/2000  |
| JP | 2001-502048 | 2/2001  |
| JP | 2002-117801 | 4/2002  |
| JP | 2002-512737 | 4/2002  |
| JP | 2003-523048 | 7/2003  |
| JP | 2003-257359 | 9/2003  |
| JP | 2007-333746 | 12/2007 |
| WO | 97/01111 A2 | 1/1997  |
| WO | 97/40381 A1 | 10/1997 |
| WO | 98/50604 A1 | 11/1998 |
| WO | 01/56055 A1 | 8/2001  |

## OTHER PUBLICATIONS

“Office Action” for JP 2010-548825, May 7, 2013, 8 pages, Japanese Patent Office, Japan.

George, Steven, M., Fabrication and Properties of Nanolaminates Using Self Limiting Surface Chemistry Techniques, Nov. 14, 2002, University of Colorado, Boulder, Colorado, US.

“Notice” for JP 2010-548825, Feb. 1, 2013, 1 page, Japanese Patent Office, Japan.

“Notice” for JP 2011-514842, Jan. 11, 2013, 1 page, Japanese Patent Office, Japan.

“Submission of Publications” for JP 2010-548825, Dec. 12, 2012, 20 pages, Japanese Patent Office, Japan.

“Submission of Publications” for JP 2011-514842, Dec. 12, 2012, 11 pages, Japanese Patent Office, Japan.

“Office Action” for Japanese Patent Application No. 2011-514842, Jun. 8, 2013, 7 pages, Japanese Patent Office.

“Notice” for JP 2010-548825, Feb. 6, 2014, 1 page, Japanese Patent Office.

Sullivan, et al., U.S. Appl. No. 13/543,804, filed Jul. 7, 2012, United States Patent Office.

Sullivan, et al., U.S. Appl. No. 13/460,726, filed Apr. 30, 2012, United States Patent Office.

“Extended Search Report” for EP Application No. 09816644.0, Jun. 5, 2014, 10 pages, European Patent Office, Munich, Germany.

“Extended Search Report” for EP Application No. 09818140.7, Jun. 5, 2014, 18 pages, European Patent Office, Munich, Germany.

Feller, W.B., et al., “Neutron Field Imaging With Microchannel Plates” Proceedings of Spie, SPIE—International Society for Optical Engineering, Jul. 31, 2000, pp. 291-302, vol. 4141, US.

Costescu, R.M., et al. “Ultra-Low Thermal Conductivity in W/A1203 Nanolaminates”, Science, American Association for the Advancement of Science, Feb. 13, 2004, pp. 989-990, vol. 303, No. 5660, US.

“Office Action” for Japanese Patent Application No. 2010-548825, May 29, 2014, 2 pages, Japanese Patent Office, JP.

“Final Office Action” for Japanese Patent Application No. 2010-548825, Dec. 19, 2014, 2 pages, Japanese Intellectual Property Office, Japan.

Tasker, et al., Microfabrication of Channel Electron Multipliers Proceedings of Spie, SPIE—International Society for Optical Engineering, Oct. 25, 1995, pp. 58-70, vol. 2640, US.

“Search Report” for European Patent Application 09758806.5, Jan. 30, 2015, 10 pages, European Patent Office, Munich, Germany.

“Examination Report” for EP 09731342.3-1556, Sep. 25, 214, 4 pages, European Patent Office, Munich, Germany.

\* cited by examiner



FIG. 1A

PRIOR ART



FIG. 1B  
PRIOR ART



FIG. 1C  
PRIOR ART



FIG. 2



FIG. 3A



FIG. 3B

FIG. 3C





FIG. 3D



FIG. 3E



FIG. 3F

## 1

MICROCHANNEL PLATE DEVICES WITH  
TUNABLE CONDUCTIVE FILMSCROSS-REFERENCE TO RELATED  
APPLICATION

This application is a continuation of U.S. patent application Ser. No. 13/460,726, entitled "Microchannel Plate Devices With Tunable Resistive Films," and filed on Apr. 30, 2012, which is a continuation of U.S. patent application Ser. No. 12/143,732, entitled "Microchannel Plate Devices With Tunable Resistive films," and filed on Jun. 20, 2008 and now U.S. Pat. No. 8,227,965. These applications are herein incorporated by reference.

## FEDERAL RESEARCH STATEMENT

This invention was made with Government support under Grant Number HR0011-05-9-0001 awarded by the Defense Advanced Research Projects Agency (DARPA). The Government has certain rights in this invention.

## BACKGROUND OF THE INVENTION

Microchannel plates (MCPs) are used to detect very low fluxes (down to single event counting) including ions, electrons, photons, neutral atoms, and neutrons. For example, microchannel plates are commonly used as electron multipliers in image intensifying devices. A microchannel plate is a slab of high resistance material having a plurality of tiny tubes or slots, which are known as pores or microchannels, extending through the slab. The microchannels are parallel to each other and may be positioned at a small angle to the surface. The microchannels are usually densely packed. A high resistance layer and a layer having high secondary electron emission efficiency are formed on the inner surface of each of the plurality of channels so that it functions as a continuous dynode. A conductive coating is deposited on the top and bottom surfaces of the slab comprising the microchannel plate.

In operation, an accelerating voltage is applied between the conductive coatings on the top and bottom surfaces of the microchannel plate. The accelerating voltage establishes a potential gradient between the opposite ends of each of the plurality of channels. Ions and/or electrons traveling in the plurality of channels are accelerated. These ions and electrons collide against the high resistance outer layer of the pore having high secondary electron emission efficiency, thereby producing secondary electrons. The secondary electrons are accelerated and undergo multiple collisions with the emissive layer. Consequently, electrons are multiplied inside each of the plurality of channels. The electrons eventually leave the channel at the output end of each of the plurality of channels. The electrons can be detected or can be used to form images on an electron sensitive screen, such as a phosphor screen or on a variety of analog and digital readouts.

## BRIEF DESCRIPTION OF THE DRAWINGS

The invention, in accordance with preferred and exemplary embodiments, together with further advantages thereof, is more particularly described in the following detailed description, taken in conjunction with the accompanying drawings. The drawings are not necessarily to scale, emphasis instead generally being placed upon illustrating principles of the invention.

## 2

FIG. 1A illustrates a perspective view of a cross section of a microchannel plate according to the prior art.

FIG. 1B illustrates a perspective view of a single channel of a microchannel plate according to the prior art.

5 FIG. 1C illustrates a cross section of a single channel of a microchannel plate according to the prior art.

FIG. 2 illustrates a cross section of a single channel of a microchannel plate according to the present invention.

10 FIG. 3A presents experimental data for resistance per channel as a function of percent CZO by ALD cycles for films deposited according to the present invention and for channel resistance of conventional microchannel plates.

FIG. 3B presents data for resistance as a function of percent copper for films fabricated according to the present invention.

15 FIG. 3C presents data for normalized microchannel plate current as a function of voltage for a commercial microchannel plate device, an intrinsic silicon microchannel plate device, and for a microchannel plate device with a nanolaminate resistive layer deposited according to the present invention.

20 FIG. 3D presents data for both microchannel plate gain and for resistance as a function of bias voltage for microchannel plates with resistive layers fabricated according to the present invention.

25 FIG. 3E presents data for relative gain as a function of dose in C/cm<sup>2</sup> for a commercial microchannel plate and for a microchannel plate with a resistive layer fabricated according to the present invention.

30 FIG. 3F presents data for normalized resistance as a function of temperature observed with the resistive film for a state-of-the-art commercial reduced lead silicate glass (RLSG) microchannel plate device, intrinsic polysilicon, and for a microchannel plate device fabricated according to the present invention.

35 Reference in the specification to "one embodiment" or "an embodiment" means that a particular feature, structure, or 40 characteristic described in connection with the embodiment is included in at least one embodiment of the invention. The appearances of the phrase "in one embodiment" in various places in the specification are not necessarily all referring to the same embodiment.

45 It should be understood that the individual steps of the methods of the present invention may be performed in any order and/or simultaneously as long as the invention remains operable. Furthermore, it should be understood that the apparatus and methods of the present invention can include any 50 number or all of the described embodiments as long as the invention remains operable.

55 The present teachings are described in more detail with reference to exemplary embodiments thereof as shown in the accompanying drawings. While the present teachings are described in conjunction with various embodiments and examples, it is not intended that the present teachings be limited to such embodiments. On the contrary, the present 60 teachings encompass various alternatives, modifications and equivalents, as will be appreciated by those of skill in the art.

65 Those of ordinary skill in the art having access to the teachings herein will recognize additional implementations, modifications, and embodiments, as well as other fields of use, which are within the scope of the present disclosure as described herein.

66 FIG. 1A illustrates a perspective view of a cross section of a microchannel plate 100 according to the prior art. The microchannel plate 100 includes a substrate 102 that defines

a plurality of pores or microchannels 104 extending from a top surface 106 of the substrate 102 to a bottom surface 108 of the substrate 102. The top surface 106 is coated with electrode material 110. The bottom surface is coated with electrode material 112. The electrode materials 110, 112 are conductive coatings that provide an electron transport medium for generating an electric field that enables cascade amplification of electrons. The microchannels 104 are hollow channels, which may be cylindrical, with channel densities that are on order of  $10^6/\text{cm}^2$  or higher.

In operation, the microchannels 104 are evacuated to pressures that are less than or equal to about  $5 \times 10^{-6}$  torr and biased by an external power supply 114. The microchannels support the generation of large electron avalanches in response to a suitable input signal. The electron multiplication process does not critically depend on either the absolute diameter (D) or length (L) of the channel, but rather on the ratio of L/D, which is sometimes referred to as  $\alpha$ . This geometric ratio largely determines the number of multiplication events (n) that contribute to the electron avalanche process. However, MCPs with smaller channel diameters tend to have slightly smaller gain than MCPs with larger channels diameters and the same L/D ratio. Typical values of  $\alpha$  range from 30 to 80 for conventional MCPs with channel diameters D on the order of 2-10  $\mu\text{m}$ .

FIG. 1B illustrates a perspective view of a single channel of a microchannel plate (MCP) 150 according to the prior art. The channel wall or dynode 160 of the MCP 150 acts as a continuous dynode for electron multiplication. The operation of the MCP 150 is similar to the operation of photo-emissive detectors using discrete dynodes (e.g., an ordinary photomultiplier tube). In operation, the dynode 160 must be sufficiently resistive to support a biasing electric field ( $\equiv$ ) $=10^2\text{-}10^5 \text{ V/cm}$  without drawing excessive current. The channel wall 160 must also be conductive enough so that a resistive layer (or strip) current is available to replenish electrons emitted from the dynode 160 during an electron avalanche. For example, when a signal event 162, such as an electrically charged particle (e.g., an electron or an ion), neutral atom/molecule or sufficiently energetic radiation (e.g., an X-ray or UV photon), strikes the channel wall 160 near the negatively biased input end 156, there is a good probability that electrons 164 will be ejected from the surface 160. These primary electrons 164 are accelerated down the channel 152 by an applied electric field  $\equiv$  produced by the bias potential ( $V_B$ ) represented by the power supply 154. The applied electric field  $\equiv$  $=V_B/L$ , where  $V_B$  in volts is about 20-25 $\alpha$  for a conventional straight-channel MCP.

Collisions of the emitted electrons 164 with the channel wall 160 cause the emission of secondary electrons 164. These secondary electrons in turn act as primary electrons in subsequent collisions with the channel wall 160 which produce another set of secondary electrons. An output electron avalanche 166 of magnitude  $\delta n$  is achieved provided that on average more than one secondary electron is emitted for every incident primary electron, e.g. secondary electron yield ( $\delta$ ) $>1$ , and n repetitions of this primary collision-secondary emission sequence in the direction of the output end 158.

FIG. 1C illustrates a cross section of a single channel 180 of a microchannel plate according to the prior art. A resistive layer 182 is formed on the outer surface of glass channel material 184. The glass channel material 184 provides mechanical support for the channel 180 in the geometry of arrays of microscopic channels within the MCP. The resistive layer 182 functions as an electronically conductive path for both discharging the emissive layer and supporting the electric fields required for the cascade amplification. An interface

layer 186 is shown to illustrate the transition from the resistive layer 182 to the emissive layer 188. A superficial silica-rich and alkali-rich (but lead-poor) dielectric emissive layer 188 (or dynode surface) that is about 2-20 nm in thickness is formed over the resistive layer 182. The emissive layer 188 produces adequate secondary emission to achieve useful electron multiplication.

Calculations indicate that a reduced lead silicate glass (RLSG) dynode including channels 180 must have a bulk electrical resistivity that is in the range of  $10^6\text{-}10^9 \Omega\text{cm}$  in order to have proper operation assuming the resistive layer 182 has a thickness  $t=100 \text{ nm}$ . Single channel electron multipliers (CEM), which are similar in construction and operation to the MCP, use only a single electron multiplication channel. This results in a resistive requirement for the CEM that is reduced by six orders of magnitude.

The microchannel plate 100 is typically manufactured using a glass multifiber draw (GMD) process. In the GMD process, individual composite fibers, consisting of an etchable core glass and an alkali lead silicate cladding glass, are formed by drawdown of a rod-in-tube perform. The rod-in-tube performs are then packed together in a hexagonal or rectangular array. This array is then redrawn into hexagonal/rectangular multifiber bundles, which are stacked together and fused within a glass envelope to form a solid billet. The solid billet is then sliced, typically at a small angle of approximately  $4^\circ\text{-}15^\circ$  from the normal to the fiber axes.

Individual slices are then polished into a thin plate. The soluble core glass is removed by a chemical etchant, resulting in an array of microscopic channels with channel densities of  $10^5\text{-}10^7/\text{cm}^2$ . Further chemical treatments, followed by a hydrogen reduction process, produces the resistive and emissive surface properties required for electron multiplication within the microscopic channels. Metal electrodes 110 and 112 are thereafter deposited on the faces of the wafer to complete the manufacture of a microchannel plate. An alternative manufacturing technique performs the draw process on the clad glass only, without core glass. This technique eliminates the need to etch the latter on the final stages.

The hydrogen reduction step is critical for the operation of prior art MCP devices and determines both the resistive and the emissive properties of the continuous dynode. Lead cations in the near-surface region of the continuous glass dynode are chemically reduced, in a hydrogen atmosphere at temperatures of  $350^\circ\text{-}650^\circ \text{ C.}$ , from the  $\text{Pb}^2$  state to lower oxidation states with  $\text{H}_2\text{O}$  as a reaction by-product. This process results in the development of significant electrical conductivity within a submicron distance to the surface of the RLSG dynode. The physical mechanism responsible for the conductivity is not well understood but is believed to be due to either an electron hopping mechanism via localized electronic states in the band gap or a tunneling mechanism between discontinuous islands of metallic lead within the RLSG film.

The observed electrical conductivity is ohmic in nature and is similar to the conductivity of a metal due to the observed material properties. The term "ohmic" means that the electrical conductivity follows Ohm's law where the resistance is substantially constant as a function of applied voltage. For example, the Temperature Coefficient of Resistance (TCR) is typically less than 1% per degree C. Also, there is an insensitivity of resistance to applied external electric field and a stability of resistance with applied bias that is observed in common metals. The presence of ohmic conduction is essential for stable MCP device operation. The resulting RLSG dynode exhibits an electrically conductive surface with a nominal sheet resistance of  $10^{14} \Omega/\text{sq}$ . It is known in the art that the electrical characteristics of RLSG dynodes represent

a complex function of the chemical and thermal history of the glass surface as determined by the details of its manufacture.

During hydrogen reduction, other high-temperature processes, such as diffusion and evaporation of mobile chemical species in the lead silicate glass (e.g., alkali alkaline earth, and lead atoms), act to modify the chemistry and structure of RLSG dynodes. Materials analysis of the near-surface region the microchannel surface of MCPs has indicated that RLSG dynodes have a two-layer structure including a resistive layer and an emissive layer as described in connection with FIG. 1C.

The RLSG manufacturing technology is mature and results in the fabrication of relatively inexpensive and high performance devices. However, the RLSG manufacturing technology has certain undesirable limitations. For example, both electrical and electron emissive properties of RLSG dynodes are quite sensitive to the chemical and thermal history of the glass surface comprising the dynode. Therefore, reproducible performance characteristics for RLSG MCPs critically depend upon stringent control over complex, time-consuming, and labor-intensive manufacturing operations. In addition, the ability to enhance or tailor the characteristics of RLSG MCPs is constrained by the limited choices of materials which are compatible with the present manufacturing technology. Performance is adversely affected by material limitations of the lead silicate glasses that are used in the manufacture of conventional MCPs. These limitations include gain amplitude and stability, count rate capabilities, maximum operating temperature, background noise, reproducibility, size, shape, and heat dissipation in high-current devices.

The manufacture of microchannel plates according to the GMD process is also limited in the choice of materials available. The multifiber drawdown technique requires that the core and cladding starting materials both be glasses with carefully chosen temperature-viscosity and thermal expansion properties. The fused billet must have properties suitable for wafering and finishing. The core material must be preferentially etched over the cladding with very high selectivity. In addition, the clad material must ultimately exhibit sufficient surface conductivity and secondary electron emission properties to function as a continuous dynode for electron multiplication. This set of constraints greatly limits the range of materials suitable for manufacturing MCPs with the present technology.

Most known microchannel plates are fabricated from glass fibers as described herein in connection with FIGS. 1A-1C. See also "Microchannel Plate Detectors," Joseph Wiza, Nuclear Instruments and Methods, Vol. 162, 1979, pages 587-601 for a detailed description of fabricating microchannel plates from glass fibers. Numerous types of substrate materials can be used for the microchannel plate 100.

Recently, silicon has been used as a substrate for microchannel plates. See, for example, U.S. Pat. No. 6,522,061 B1 to Lockwood, which is assigned to the present assignee. Silicon microchannel plates have several advantages compared with glass microchannel plates. Silicon microchannel plates can be more precisely fabricated because the channels can be lithographically defined rather than manually stacked like glass microchannel plates. Silicon processing techniques, which are very highly developed, can be applied to fabricating such microchannel plates. Also, silicon substrates are much more process compatible with other materials and can withstand high temperature processing.

In contrast, glass microchannel plates melt at much lower temperatures than silicon microchannel plates. Furthermore, silicon microchannel plates can be easily integrated with

other devices. For example, a silicon microchannel plate can be easily integrated with various types of other electronic and optical devices, such as photodetectors, MEMS, and various types of integrated electrical and optical circuits. One skilled in the art will appreciate that the substrate material can be any one of numerous other types of insulating substrate materials.

Also, U.S. Pat. No. 5,378,960 entitled "Thin Film Continuous Dynodes For Electron Multiplication" to Tasker teaches that the current carrying layer of the RLSG dynode of prior art 10 MCP devices can be replaced with a semiconducting, current carrying layer, such as a Si or Ge semiconductor layer, doped semiconductors (P-doped Si), silicon-oxides ( $\text{SiO}_x$ ) or silicon nitrides ( $\text{Si}_x\text{N}_y$ ). U.S. Pat. No. 5,378,960 also describes that the MCP current carrying layer must have a resistivity in the 15 range of  $10^6$ - $10^9 \Omega\text{-cm}$  for nominal 100 nm films, which corresponds to a sheet resistance of  $10^{11}$ - $10^{14} \Omega/\text{sq}$ . This value of sheet resistance is necessary in order to sustain the MCP bias voltage, which for an L/D of 40:1 must be about 1,000V, with optimized current draw so that the device can be 20 recharged with sufficient speed without excess power dissipation. In fact, commercially available MCP devices, such as those used in charged particle detectors and image intensifier tubes require the sheet resistances to be greater than  $10^{14} \Omega/\text{sq}$  for many applications.

25 The resistivity of pure Si is about  $2.3 \times 10^5 \Omega\text{-cm}$  assuming the maximum possible resistance value for the pure semiconducting materials as the value obtained with the intrinsic carrier concentration (e.g. undoped). Similarly, the resistivity of pure Ge is about  $47 \Omega\text{-cm}$  assuming the maximum possible 30 resistance value for the pure semiconducting materials as the value obtained with the intrinsic carrier concentration (e.g. undoped). Thus, the maximum sheet resistance for an MCP device (assuming a minimum, viable, film thickness of 100 nm) is  $5.8 \times 10^{10} \Omega/\text{sq}$  for Si and is  $2 \times 10^7 \Omega/\text{sq}$  for Ge, which 35 are both several orders of magnitude below the sheet resistance required for stable MCP operation. By stable operation we mean an operating mode where the MCP is not generating excess Joule heat that causes thermal runaway due to a negative temperature coefficient of resistance. Consequently, 40 these Si and Ge films are suited only for the CEM class of electron multipliers.

Another fundamental limitation on the use of semiconducting thin films as the current carrying layer for CEMs and MCPs is the susceptibility of these thin films to electric fields.

45 Applying an electric field transverse to the direction of current conduction results in a characteristic which is similar to that of the field effect transistors (FETs). The field effect in CEMs and MCPs devices causes modulation of the conductivity of the semiconducting layer due to the external applied field. More specifically, during the operation of a MCP channel, positive charge builds up on the emissive film surface due to the departure of secondary electrons during the amplification cascade process. This positive charge sets up a relatively 50 strong electric field across the thin emissive film which serves to decrease the resistance of the underlying, intrinsic current carrying layer, by increasing the concentration of carriers (electrons) at the interface between the resistive layer and the emissive layer (shown as the interface 186 FIG. 1C). This 55 effect is readily measured in MCP devices including a resistive layer formed of a semiconducting material by observing changes in the current which flows through the device as a function of applied input. The field effect in semiconductors results in a device resistance that is not stable. This instability in the device resistance is independent of doping levels.

60 The increased carrier concentration can result in a resistance decrease of several orders of magnitude within the current carrying layer. Semiconducting films also show large

values of resistance change with temperature or Temperature Coefficient of Resistance (TCR). For intrinsic Si, the TCR is as high as 8% per degree C. as compared with less than 1% per degree C. for the RLSG films found in prior art glass MCP devices. The low maximum resistance of the semiconducting films (four orders of magnitude below prior art glass MCPs) and the high resulting current draw when combined with the field effect (which in MCP operation results in a further lowering of the layer resistance and increase in current draw) results in an MCP device that will not function with a stable resistance. Such an MCP may experience thermal runaway due to the relatively high Joule heating that is positively reinforced by the high negative value of the TCR. For these reasons, the semiconducting films are not suitable for the MCP device.

Also, U.S. Pat. No. 5,378,960 describes the use of oxides and nitrides of semiconductors as a conduction layer. Conduction within oxides and nitrides of semiconductors, such as  $\text{SiO}_x$  and  $\text{Si}_x\text{N}_y$ , is achieved through one of four mechanisms: Fowler-Nordheim tunneling; Poole-Frenkel conduction; space charge limited conduction; and ballistic transport. Space charge limited conduction and ballistic transport can not occur in MCP devices because they require very high currents (space charge  $\sim V^2$ ) or very high fields (ballistic  $\sim V^{1.5}$ ).

It is well known that electrons can travel through a thin  $\text{SiO}_2$  film by means of direct tunneling or Fowler-Nordheim (F-N) tunneling. Direct tunneling indicates the presence of a trapezoidal potential barrier whereas F-N tunneling takes place when electrons tunnel through a potential barrier which is triangular in shape. Direct tunneling requires an extremely thin dielectric layer (thin in the direction of the applied field) of about 4 nm or less for  $\text{SiO}_2$ . In MCPs the effective thickness of the conduction layer in the direction of the applied field is typically several hundred microns. A large electric field is typically needed for F-N tunneling in order to transform a rectangular potential barrier to a triangular potential barrier. Therefore, Fowler-Nordheim tunneling usually dominates in relatively high electric fields while direct tunneling is the main conduction mechanism for thin films in low electric fields.

The Frenkel-Poole effect has also been observed in  $\text{SiO}_2$ , even though tunneling is considered to be mainly responsible for charge transport in  $\text{SiO}_2$ . The Frenkel-Poole effect relates to the electric field enhanced thermal emission of charge carriers from charged traps. It is known that Si traps can be charged. Thus, it is possible that Si traps can efficiently emit charge carriers in silicon oxide with an applied electric field.

The current conduction mechanism in silicon nitride is well known. Typically current conduction in silicon nitride is a defect-assisted current conduction mechanism that is dominated by electrons jumping between geometrically close defects. This mechanism is described by the Frenkel-Poole equation.

For both  $\text{SiO}_x$  and  $\text{Si}_x\text{N}_y$ , current carrying layers, the electric fields required to supply the appropriate leakage current to support the channel emissive layer re-charge is at least two orders of magnitude higher ( $10^6$  vs.  $10^4$  V/cm) than the known MCP bias supplies are capable of providing (1,000V vs. 100,000V). Bias voltages of 100,000V are not practical for the typical MCP application. Also, these high voltages will substantially increase the mean free path of the electrons within the channel. In addition, these high voltages will significantly reduce the number of collisions, and significantly reduce the resulting gain of the device. For these reasons, silicon oxide and silicon nitride based films will not function as resistive films for the MCP applications.

U.S. Pat. No. 7,097,526 entitled "Method of Forming Nitrogen and Phosphorus Doped Amorphous Silicon as Resistor for Field Emission Display Device Baseplate" to Raina describes using nitrogen or oxygen doping of silicon to increase the thin film resistance. This patent states that it is possible to change the conductivity of bulk amorphous silicon over a range of 500 to  $10^4$   $\Omega\text{-cm}$  by varying the nitrogen doping. Similarly, U.S. Pat. No. 6,268,229 entitled "Integrated Circuit Devices and Methods Employing Amorphous Silicon Carbide Resistor Materials" to Brandes et al. describes that amorphous silicon-carbide, through selection of the silicon-to-carbide ratio and concentrations of various dopants, can demonstrate resistivity in a range from 1  $\Omega\text{-cm}$  to  $10^{11}$   $\Omega\text{-cm}$ . While it has been demonstrated that these films are capable of achieving the resistivity required for MCP operation, the films remain semiconducting and subject to the same problems as semiconductors. Moreover, the high resistivity range of those films was found to be very hard to reproduce between different experimental runs due to their extremely high sensitivity to any impurities, dopants, and grain various dimensions.

The present invention relates to microchannel plate devices with continuous dynodes having widely tunable conductivity during fabrication. In one embodiment, the resistance of layers can be tuned over a range from about  $10^9$ - $10^{16}$   $\Omega/\text{sq}$ . Film layers can also have electrical conductivity essentially similar to the ohmic electrical conductivity of metals. Films can also have a conductivity that is not affected by an applied external transverse electric field, a relatively small TCR value, and a resistance value that is stable as a function of applied bias.

In various embodiments of the present invention, the resistive layer, either alone or in conjunction with at least an emissive layer, are formed in each of the plurality of channels of the microchannel plates by various deposition techniques, such as atomic layer deposition. One skilled in the art will appreciate that the methods of the present invention can be used with any type of microchannel plate substrate including conventional glass microchannel plates, semiconductor microchannel plates, and ceramic microchannel plates.

Each of the plurality of channels in the microchannel plate according to the present invention includes at least a resistive and an emissive layer or a combined emissive/resistive layer. Microchannel plates according to the present invention can include a resistive layer combined with any number of emissive layers formed on the channels. In various embodiments, other resistive layers can be formed on the outer surface of the plurality of channels, between emissive layers, and/or on the outer surface of the outer emissive layer. Also, in various embodiments, thin resistive layers can be formed on the outer surface of the plurality of channels, between emissive layers, and/or on the outer surface of the outer emissive layer. Various possible resistive and emissive layers are described in more detail in connection with FIG. 2.

FIG. 2 illustrates a cross section of a single channel 280 of a microchannel plate according to the present invention. A resistive layer 282 is formed on the outer surface of the channel 280, whose resistance can be tuned to achieve a predetermined level of conductivity during fabrication. In some embodiments, the resistive layer 282 is a nanolaminate structure, containing alternating thin films comprised of  $\text{Al}_2\text{O}_3$  insulating layers stacked with zinc doped copper oxide nanoalloy (CZO) conducting films. Materials that comprise the conducting and insulating layers can be selected, for example, based upon the bandgap of candidate materials. Candidate materials can be divided into three primary groups, based upon bandgap: no-bandgap (metals), moderate bandgap (semi-conducting/semi-insulating), and large bandgap

(insulators). For example, the no-bandgap materials can include: Ru, Rh, Pd, Re, Os, Ir, Pt, and Au. The moderate bandgap materials can include oxides of Zn, V, Mn, Ti, Sn, Ru, In, Cu, Ni, and Cd. The large bandgap materials can include oxides and nitrides of Al, Si, Mg, Sn, Ba, Ca, Sr, Sc, Y, La, Zr, Hf, Ta, Ti, V, Cs, B, Nb, Be, and Cr.

In various other embodiments, the conducting layer of the nanolaminate resistive layer 282 is formed using mid-bandgap materials, such as oxides of Zn, V, Mn, Ti, Sn, Ru, In, Cu, Ni, and Cd. The conducting layer can include any insulating oxide or nitride (large bandgap materials) doped with metallic (no-bandgap materials) species, such as Ru, Rh, Pd, Re, Os, Ir, Pt, and Au. In various embodiments, the insulating film used in the nanolaminate resistive layer 282 can be formed using very large bandgap materials, such as oxides and nitrides of: Al, Si, Mg, Sn, Ba, Ca, Sr, Sc, Y, La, Zr, Hf, Ta, Ti, V, Cs, B, Nb, Be, and Cr, and any mixture thereof. The nanolaminate structure can also include a resistive film, which can be a metal oxide alone or a nanoalloy. The resistive film can also be a doped semi-insulating oxide or a pure semi-insulating oxide.

The term "nanolaminate" is defined herein as a composite film of ultra thin layers of two or more materials in a layered stack, where the layers are alternating layers of materials of the composite film. For extremely thin alternating layers, the term "nanoalloy" is often used. However, the distinction between the term "nanolaminate" and the term "nanoalloy" is not clear in the art. The term "nanoalloy" as used herein describes films formed from extremely thin nanolaminates, which are no more than a few monolayers thick. Typically, each layer in a nanolaminate has a thickness in the few Angstrom range up to several nanometers. Each individual material layer of the nanolaminate can have a thickness that is as thin as a monolayer of the material.

For example, a nanolaminate of zinc doped copper oxide nanoalloy (CZO) and aluminum oxide includes at least one thin layer of CZO, and one thin layer of the aluminum oxide. Such a layer can be described as a nanolaminate of CZO/aluminum oxide. A CZO/aluminum oxide nanolaminate is not limited to alternating one CZO layer after an aluminum oxide layer, but can include multiple thin layers of CZO alternating with multiple thin layers of aluminum oxide. Furthermore, the number of thin layers of CZO and the number of thin layers of aluminum oxide can vary independently within a nanolaminate structure.

Additionally, CZO/aluminum oxide nanolaminate can include layers of different conducting and insulating oxides, where each layer is selected according to its insulating or conducting properties. A dielectric layer containing alternating layers of conducting oxides and insulating oxides has an effective conductivity that is related to the combination of the layers of the nanolaminate. The value of the effective conductivity depends on the relative thicknesses of the conducting oxide layers and the insulating oxide layers. Thus, such a film containing a conducting oxide/insulating oxide nanolaminate can be engineered to effectively provide a predetermined resistance that can be varied over a wide range during fabrication.

The conductivity of the dynode film can also be modulated by doping the conducting film. The zinc doped copper oxide nanoalloy is an example of such a film, where the zinc content of the zinc doped copper oxide nanoalloy can be used to determine the conductivity of the zinc doped copper oxide nanoalloy. Thus doping may be used alone, or in conjunction with the nanolaminate, to engineer a selected film resistance.

In some embodiments, a thin barrier layer 284 is formed on the outer surface of the channel 280 before the first resistive

layer 282 is formed. The thin barrier layer 284 can also be used to improve or to optimize MCP device functions, such as secondary electron emission, gain, uniformity, lifetime, and/or process yield. The thin barrier layer 284 can also be used to achieve a predetermined current output of the microchannel plate. The thin barrier layer 284 can also be used to control charge trapping characteristics of the MCP. In addition, the thin barrier layer 284 can be used to passivate the outer surface of the channel 280 to prevent ions from migrating out of the surface of the channel 280.

The electrostatic fields maintained within the microchannel plate that move electrons through the channel 280 also move any positive ions that migrate through the channel 280 towards a photocathode or other up-stream device or instrument used with the microchannel plate. These positive ions include the nucleus of gas atoms which can be of considerable size, such as hydrogen, oxygen, and nitrogen. These gas atoms are much more massive than electrons. Such positive gas ions can be accelerated toward the channel entrance and even farther to impact other components which may be used in concert with the MCP. An example of such a device is the image intensifier tube component of night vision devices which uses a photocathode (typically GaAs) to generate electrons which are amplified by the MCP to provide low light imaging. Ion impact upon the photocathode causes physical and chemical damage. Other gas atoms present within the channel 280 or proximate to the photocathode may destroy the negative electron affinity of the photocathode required for high efficiency and/or may be effective to chemically combine with and poison the photocathode.

In addition, the channel 280 includes an emissive layer 288 that is formed over the resistive layer 282 or over the barrier layer 286. In various embodiments, the emissive layer 288 comprises oxides and nitrides of at least one element selected from the group consisting of: Al, Si, Mg, Sn, Ba, Ca, Sr, Sc, Y, La, Zr, Hf, Ta, Ti, V, Cs, B, Nb, Be, Cr, and any mixture thereof. In some embodiments, the thickness and material properties of the emissive layer 288 are generally chosen to increase the secondary electron emission efficiency of the microchannel plate compared with conventional microchannel plates fabricated with the lead-glass, multi-draw process. In some embodiments, the thickness and material properties of the emissive layer 288 are generally chosen to provide a barrier to ion migration. Such a barrier to ion migration can be used to control charge trapping characteristics.

FIG. 2 illustrates a microchannel plate with resistive and emissive layers 282, 288. However, one skilled in the art will understand that microchannel plates can be fabricated according to the present invention with any number and combination of resistive and emissive layers. In such embodiments, there are many possible combinations of different emissive and resistive layer compositions and thicknesses. In addition, the multiple resistive and emissive layers can be stacked with or without barrier layers.

Experiments have shown that depositing resistive films by atomic layer deposition (ALD) significantly enhances the performance of the microchannel plate. Atomic layer deposition has been shown to be effective in producing highly uniform, pinhole-free films having thicknesses that are as thin as a few Angstroms. Films deposited by ALD have relatively high quality and high film integrity compared with other deposition methods, such as physical vapor deposition (PVD), thermal evaporation, and chemical vapor deposition (CVD), especially taking into account large aspect ratios of MCP pores.

Atomic Layer Deposition (ALD) is a chemical process used to create extremely thin coatings. Atomic layer deposi-

## 11

tion is a variation of CVD that uses a self-limiting reaction. The term “self-limiting reaction” is defined herein to mean a reaction that limits itself in some way. For example, a self-limiting reaction can limit itself by terminating after a reactant is completely consumed by the reaction or once the reactive sites on the deposition surface have been occupied.

A cycle of an ALD deposition sequence includes pulsing a precursor material, pulsing a purging gas for the precursor material, pulsing a reactant precursor, and pulsing the reactant’s purging gas. The result of an ALD deposition sequence is a very consistent deposition thickness that depends upon the amount of the first precursor that adsorbs onto and then saturates the surface. This cycle can be repeated until the desired thickness is achieved in a single material layer. This cycle can also be alternated with pulsing a third precursor material, pulsing a purging gas for the third precursor, pulsing a fourth reactant precursor, and pulsing the reactant’s purging gas. In some methods of the present invention, there does not need to be a reactant gas if the precursor material interacts with the substrate directly. For example, in one embodiment of the present invention, the ALD deposition sequence includes pulsing dopant metal precursor material onto a conducting oxide layer.

Nanolayer and nanolaminate materials are composite materials that include ultra-thin layers of two or more different materials in a layered stack, where the layers are alternating layers of different materials having a thickness that is on the order of a nanometer or less. Nanolayer and nanolaminate materials may be continuous films that are a single monolayer thick. Nanolayer and nanolaminate materials are formed when the thickness of the first series of cycles results in a layer that is only a few molecular layers thick, and the second series of cycles results in a different layer that is only a few molecular layers thick.

Nanolayer and nanolaminate materials are not limited to alternating single layers of each material. Instead, nanolayer and nanolaminate materials can include several layers of one material alternating with a single layer of the other material that form a desired ratio of the two or more materials. Such an arrangement can achieve a film having a conductivity that varies over a wide range. Nanolayer and nanolaminate materials can also include several layers of one material formed by an ALD reaction either over or under a single layer of a different material formed by another type of reaction, such as a MOCVD reaction. The layers of different materials may remain separate after deposition, or they may react with each other to form an alloy layer. The alloy layer can be a doping layer. Doping the layer can be used to vary the properties of the layer.

Nanolaminate zinc-doped copper oxide (CZO) films can be formed by ALD deposition using an alkyl-type precursor chemical, such as DEZ, an acetonate-type precursor, such as Cu(hfac)<sub>2</sub>, and an oxidizing precursor, such as DI water. Such films can be formed at relatively low temperatures, which can be 250° C. or lower. Such films can be amorphous or polycrystalline and possess smooth surfaces. Such films may provide enhanced electrical properties as compared to films formed with physical deposition methods, such as sputtering, or typical chemical layer depositions, due to their relatively smooth surface and reduced damage which results in more repeatable electrical performance.

In one embodiment, a CZO/Al<sub>2</sub>O<sub>3</sub> nanolaminate resistive layer is formed using atomic layer deposition (ALD). Such a film has a relatively smooth surface relative to other processing techniques. The transitions can be controlled during the formation of such a film by using atomic layer deposition. Thus, the deposited CZO/Al<sub>2</sub>O<sub>3</sub> nanolaminate layers can be

## 12

engineered to provide the required electrical or physical characteristics. In addition, the ALD deposited CZO/Al<sub>2</sub>O<sub>3</sub> nanolaminate layers provide conformal coverage on the surfaces on which they are deposited.

5 Another aspect of the microchannel plates of the present invention is that the resistive layer 282 and any other resistive and emissive layers formed on the substrate 280 protect and passivate the substrate 280. That is, the resistive layer 288 and any other resistive and conductive layers formed on the substrate layer 280 can provide a barrier to ion migration that can be used to control outgassing characteristics. Resistive and emissive layers are easily damaged.

In glass microchannel plates, the alkaline metals contained in the Pb-glass formulation are relatively stable in the bulk material. However, alkaline metals contained in the reduced lead silicate glass (RLSG) on the outer surface of the microchannels which forms the emissive layer are only loosely held within the film structure because of their exposure to the high temperature hydrogen environment that removes oxygen and breaks bonds in material structure. The electron bombardment that occurs during electron multiplication erodes these elements from the film. This erosion degrades the gain of the microchannel plate over time. In silicon microchannel plates, the emissive layer is typically a very thin coating that also erodes during electron bombardment which occurs during normal device operation. One aspect of the present invention is that resistive and emissive can be engineered to better withstand the effects of electron bombardment.

Thus, in various embodiments, at least one of a thickness 30 and a composition of the resistive layer can be chosen to passivate the microchannel plate so that the number of ions released during initial operation (outgassing of ion species, such as H, CO, CO<sub>2</sub>, and H<sub>2</sub>O) as well as longer term removal of adsorbed alkali metals, such as Na, K, and Rb from the 35 substrate is reduced. Reducing the number of ions released from the substrate will improve the lifetime of the microchannel plate as well as the lifetime of devices which utilize the MCP in combination with a photocathode. Photocathodes are particularly susceptible to ion poisoning from outgassed or 40 desorbed ions from the MCP. Choosing the thickness and the composition of the resistive layer to passivate the microchannel plate substrate will also improve the process yield.

Another aspect of the microchannel plates of the present invention is that the resistive and emissive layers 282, 288 can 45 be optimized independently of each other. The resistive and emissive layers 282, 288 can also be optimized independently of other microchannel plate parameters to achieve various performance, lifetime, and yield goals. For example, the resistive layer 282 can be optimized to enable a specific 50 output current operating range. The secondary electron emission layers 288 can be optimized separately to achieve high or maximum secondary electron emission efficiency or high or maximum lifetime and/or have high count rate capabilities. Such a microchannel plate can have significantly improved 55 microchannel plate gain, count rate, and lifetime performance compared with prior art microchannel plate devices.

The ability to independently optimize the various resistive and emissive layers is important because the performance of microchannel plates is determined by the properties of these 60 combined layers that form the continuous dynodes in the channels. The continuous dynodes must have emissive and resistive surface properties that provide at least three different functions. First, the continuous dynodes must have emissive surface properties desirable for efficient electron multiplication. Second, the continuous dynodes must have conductive properties that allow the emissive layer to support a current 65 adequate to replace emitted electrons. Third, the continuous

dynodes must have resistive properties that allow for the establishment of an accelerating electric field for the emitted electrons.

Consequently, the performance of these three functions: emitting secondary electrons; replacing emitted electrons; and establishing an accelerating electric field for the emitted electrons, can not typically be simultaneously maximized within the current, state-of-the-art MCP technology that utilizes a single, combined RLSG resistive and emissive layer. Thus, in prior art single emissive layer microchannel plate devices, the secondary emission properties of the emissive layer can not be optimized to maximize secondary electron emission and, therefore, can not be optimized to maximize the sensitivity performance of the microchannel plates. In fact, most known microchannel plates are fabricated to optimize the resistance of the device over a very narrow range that is determined by the macroscopic material composition of the glass, rather than to optimize the secondary electron emission. The method of the present invention allows the various resistive and emissive layers to be independently optimized for one or more performance, lifetime, or yield goal.

FIG. 3A presents experimental data 300 for resistance per channel as a function of percent CZO by ALD cycles for films deposited according to the present invention and for channel resistance of conventional microchannel plates. Resistance per channel data 302 for conventional microchannel plates is presented for conventional state-of-the-art microchannel plates having a single, combined resistive and emissive layer. The data 302 indicates that the resistance per channel is about  $10^{14}$ . These data were taken for a manufactured microchannel plate device that is commonly used in state-of-the-art night vision devices.

FIG. 3A also presents data 304 for resistance per channel as a function of percent CZO by ALD cycles for an alternating combination of  $(\text{CZO}/\text{Al}_2\text{O}_3) \times N$  layers of resistive films deposited according to the present invention. In addition, data 306 is presented for resistance per channel as a function of percent CZO by ALD cycles for an alternating combination of CZO $\times 2$  layers/ $\text{Al}_2\text{O}_3 \times N$  layers resistive film deposited according to the present invention.

In order to present a fair comparison, the data 304, 306 was obtained for the same conventional microchannel plate devices with the resistance per channel data 302 shown in FIG. 3A, but where processing was terminated immediately prior to the hydrogen reduction step that would have resulted in the simultaneous formation of the resistive and emissive layers. Resistive and emissive layers were then formed according to the present invention. The data 300 demonstrates the wide possible range of channel conductivity that can be achieved using the methods of the present invention compared with prior art microchannel plate fabrication methods.

FIG. 3B presents data 320 for resistance as a function of percent copper for films fabricated according to the present invention. Data 322 is presented for zinc doped copper oxide (CZO) films. The data 322 indicate that by modulating the percent of zinc contained in the zinc doped copper oxide film according to the present invention, it is possible to vary the resistance over nearly two orders of magnitude. Data 324 is also presented for CZO/ $\text{Al}_2\text{O}_3$  nanolaminate films fabricated according to the present invention. The data 324 indicate that by fixing the percentage of zinc within the CZO film and by varying the CZO/ $\text{Al}_2\text{O}_3$  nanolaminate ratios according to the present invention, it is possible to achieve a much wider range of resistivity. The range in this experiment is limited by test structure design, to an upper value which is much less than that shown in FIG. 3A.

FIG. 3C presents data 330 for normalized microchannel plate current as a function of voltage for a commercial RLSG microchannel plate device, an intrinsic silicon microchannel plate device, and for a microchannel plate device with a nanolaminate resistive layer deposited according to the present invention. Normalized current-voltage data 332 is presented for a commercial RLSG microchannel plate device. Normalized current-voltage data 334 is presented for a microchannel plate device with a nanolaminate resistive layer deposited according to the present invention.

The normalized current-voltage data 332 for the commercial RLSG microchannel plate and the normalized current-voltage data 334 for the microchannel plate device with the nanolaminate resistive layer deposited according to the present invention shows a nearly identical linear normalized current-voltage characteristic. The nearly linear data characteristic suggests that both the commercial device and the device with the nanolaminate resistive layer according to the present invention demonstrate ohmic behavior by possessing a nearly identical and substantially constant resistance as a function of applied voltage. The inherent stability of resistance of the nanolaminate resistive layer deposited according to the present invention is due to the ability to tailor the conduction of the resistive layer using the combined nanolaminate/nanoalloy microstructure described herein.

Normalized current-voltage data 336 is presented for an intrinsic silicon microchannel plate device. The non-ohmic behavior shown by the data 336 suggests that the intrinsic silicon microchannel plate shows a resistance that is not substantially constant as a function of applied voltage, which can be attributed to thermal and electric field effects which alter the conductivity of the semiconducting intrinsic silicon dynode.

FIG. 3D presents data 350 for both microchannel plate gain and for resistance as a function of bias voltage for microchannel plates with resistive layers fabricated according to the present invention. The microchannel plate devices include channels having a diameter that is about 5 microns and an L/D ratio that is equal to about 50:1. The data were acquired by varying the bias voltage from 500 to 1,000V with a constant input current.

Data 352 is presented for microchannel plate resistance as a function of bias voltage for a microchannel plate with resistive layers fabricated according to the present invention. Data 354 is presented for microchannel plate gain as a function of bias voltage for a microchannel plate with a resistive layer fabricated according to the present invention. The data 352, 354 indicate that the microchannel plate devices according to the present invention achieve a stable resistance across the operating voltage and a higher gain for equivalent bias and input conditions compared with prior art microchannel plate devices.

FIG. 3E presents data 370 for relative gain as a function of dose in  $\text{C}/\text{cm}^2$  for a commercial RLSG microchannel plate and for a microchannel plate with a resistive layer fabricated according to the present invention. Data 372 is presented for relative gain data as a function of the total extracted charge density in  $\text{coulombs}/\text{cm}^2$  for the commercial RLSG microchannel plate. Data 374 is presented for relative gain data as a function of the total extracted charge density in  $\text{coulombs}/\text{cm}^2$  for a microchannel plate with a resistive layer fabricated according to the present invention.

The data 372, 374 demonstrate the enhanced lifetime observed with the combined resistive and emissive films fabricated according to the present invention, as compared with lifetime data collected using present state-of-the-art microchannel plate technology. The relative gain degradation data

## 15

indicate that there is significantly less gain degradation for microchannel plates having a resistive and emissive layer fabricated according to the present invention as a function of the total extracted charge. Thus, the gain degradation data indicate that fabricating the resistive and emission layers according to the present invention can significantly improve microchannel plate device lifetimes.

FIG. 3F presents data 390 for normalized resistance as a function of temperature observed with the resistive film for a state-of-the-art commercial reduced lead silicate glass (RLSG) microchannel plate device, intrinsic polysilicon, and for a microchannel plate device fabricated according to the present invention. Data 392 is presented for the resistive film for a state-of-the-art commercial RLSG microchannel plate device. Data 394 is presented for intrinsic polysilicon. Data 396 is presented for a microchannel plate device fabricated according to the present invention.

The data 392 and 396 indicate that the temperature coefficient of resistance for the microchannel plate device fabricated according to the present invention is comparable to the temperature coefficient of resistance for the commercial RLSG microchannel plate device. The temperature coefficient of resistance of both the present invention and the RLSG device is less than 1% per degree C., which exhibits ohmic or "metallic" conduction behavior that significantly exceeds the temperature coefficient of resistance performance of the intrinsic polysilicon, which is more than 8% per degree C.

## EQUIVALENTS

While the present teachings are described in conjunction with various embodiments and examples, it is not intended that the present teachings be limited to such embodiments. On the contrary, the present teachings encompass various alternatives, modifications and equivalents, as will be appreciated by those of skill in the art, which may be made therein without departing from the spirit and scope of the invention.

## What is claimed is:

1. A microchannel plate detector comprising: a substrate having a plurality of channels extending from a top surface of the substrate to a bottom surface of the substrate; a resistive layer having a resistance that is substantially constant as a function of applied voltage over an operating range of the microchannel plate detector, the resistive layer being formed by conformal deposition over the outer surface of the plurality of channels; and at least one electron emissive layer formed by conformal deposition over the resistive layer.

2. The microchannel plate of claim 1, wherein the resistive layer consists of an alternating sequence of insulating and conducting layers.

3. The microchannel plate of claim 2, wherein the conducting layers are comprised of candidate materials with no bandgap, interspersed within a large bandgap material.

4. The microchannel plate of claim 3, wherein the resistive layer comprises a nanoalloy.

5. The microchannel plate of claim 2, wherein the conducting layers comprise alternating layers of lower bandgap material higher bandgap material.

6. The microchannel plate of claim 5, wherein the resistive layer comprises a nanolaminate.

7. The microchannel plate of claim 1 wherein a Temperature Coefficient of Resistance (TCR) of the resistive layer is less than one percent.

8. The microchannel plate of claim 1, wherein the resistive layer and electron emissive layer provide a relative current gain for the microchannel plate that is greater than approxi-

## 16

mately 0.6 over an incident dose ranging between approximately 0.001 C-cm<sup>-2</sup> and approximately 0.015 C-cm<sup>-2</sup>.

9. The microchannel plate of claim 1, wherein the resistive layer and electron emissive layer provide a relative current gain for the microchannel plate that is greater than approximately 0.8 over an incident dose ranging between approximately 0.001 C-cm<sup>-2</sup> and approximately 0.015 C-cm<sup>-2</sup>.

10. The microchannel plate of claim 5, wherein the resistance of the resistive layer is substantially constant between the bias voltage values of approximately 500 volts and approximately 1,000 volts.

11. The microchannel plate of claim 1, wherein a resistance of the resistive layer is determined by at least a dopant concentration within the resistive layer.

12. The microchannel plate of claim 1, wherein a resistance of the resistive layer is determined by at least one layer thickness within the resistive layer.

13. The microchannel plate of claim 1, wherein a resistance of the resistive layer is determined by at least a number of layers within the resistive layer.

14. The microchannel plate of claim 1, wherein a resistance of the resistive layer is determined by a ratio of conductive to insulating layers within the resistive layer.

15. A method for making a microchannel plate detector, the method comprising: forming by conformal deposition a resistive layer over the outer surface of a plurality of channels that extend through a substrate; selectively tuning a resistivity of the resistive layer so that a resistance of the resistive layer is substantially constant as a function of applied voltage over an operating range of the microchannel plate detector; and forming, by conformal deposition, an electron emissive layer over the resistive layer.

16. The method of claim 15, further comprising forming the resistive layer by an alternating sequence of insulating and conducting layers.

17. The method of claim 16, further comprising forming the conducting layers by conformal deposition of candidate materials with no bandgap, interspersed within a large bandgap material.

18. The method of claim 17, further comprising forming the resistive layer by conformal deposition of a nanoalloy.

19. The method of claim 15, further comprising forming the conducting layers by conformal deposition of candidate materials with moderate bandgap in alternating layers with a large bandgap material.

20. The method of claim 19, further comprising forming the resistive layer by conformal deposition of a nanolaminate.

21. The method of claim 15, further comprising forming the resistive layer for which the Temperature Coefficient of Resistance (TCR) is less than one percent.

22. The method of claim 15, further comprising forming the resistive layer and electron emissive layer to provide a relative current gain for the microchannel plate that is greater than 0.6 over an incident dose ranging between approximately 0.001 C-cm<sup>-2</sup> and 0.015 C-cm<sup>-2</sup>.

23. The method of claim 15, wherein forming the resistive layer and electron emissive layer to provide the relative current gain comprises controlling at least one of a thickness of a layer within the resistive layer, a dopant concentration of at least one layer within the resistive layer, a ratio of conductive to insulating layers within the resistive layer, or a thickness of the resistive layer.

24. The method of claim 15, further comprising forming the resistive layer and electron emissive layer to provide a relative current gain for the microchannel plate that is greater than 0.8 over an incident dose ranging between approximately 0.001 C-cm<sup>-2</sup> and 0.015 C-cm<sup>-2</sup>.

**17**

**25.** The method of claim **15**, further comprising forming the resistive layer to provide a resistance that is constant between the bias voltages values of approximately 500 volts and 1,000 volts.

**26.** The method of claim **15**, wherein selectively tuning the resistivity comprises controlling a dopant concentration within the resistive layer to set the resistivity of the resistive layer to a selected value.

**27.** The method of claim **15**, wherein selectively tuning the resistivity comprises controlling at least one layer thickness within the resistive layer to set the resistivity of the resistive layer to a selected value.

**28.** The method of claim **15**, further comprising controlling a number of layers within the resistive layer to set a resistance of the resistive layer to a selected value.

**29.** The method of claim **15**, wherein selectively tuning the resistivity comprises controlling a ratio of conductive to insu-

5 lating layers within the layer to set the resistivity of the resistive layer to a selected value.

**30.** A microchannel plate comprising:

- a) a substrate defining a plurality of channels extending from a top surface of the substrate to a bottom surface of the substrate;
- b) a resistive layer comprising a nanolaminate structure formed over an outer surface of the plurality of channels, the nanolaminate structure being chosen to have a composition that provides ohmic conduction with a predetermined resistivity that is substantially constant over an operating range of the microchannel plate detector;
- c) an emissive layer formed over the resistive layer; and
- d) a top electrode positioned on the top surface of the substrate; and a bottom electrode positioned on the bottom surface of the substrate.

\* \* \* \* \*